

Patented Nov. 19, 1935

2,021,782

# UNITED STATES PATENT OFFICE

2,021,782

## ALLOY STEEL AND ARTICLES MADE THEREFROM

Walter G. Hildorf, Canton, Ohio, and Albert E. White and Claude L. Clark, Ann Arbor, Mich., assignors to The Timken Roller Bearing Company, Canton, Ohio, a corporation of Ohio, as trustee

No Drawing. Application November 20, 1931,  
Serial No. 576,429

5 Claims. (Cl. 75—1)

Our invention relates to alloy steels which are required to withstand stresses of considerable magnitude at elevated temperatures that is above 750° F., which is resistant to oxidation at such temperatures and which is considerably lower in cost than the austenitic steels or chromium steels, commonly used at such temperatures.

10 The principal object of our invention is an alloy steel suitable for use at such high temperatures but containing sufficiently small amounts of alloying elements to make the cost of the steel comparable to that of simple alloy steels.

15 The invention consists principally in a chromium-tungsten-silicon steel, with or without vanadium, having substantially the following composition:

|             | Per cent     |
|-------------|--------------|
| 20 Carbon   | 0.20 to 0.60 |
| Manganese   | 0.20 to 1.0  |
| Silicon     | 0.50 to 1.0  |
| Chromium    | 0.75 to 1.50 |
| Tungsten    | 0.50 to 1.50 |
| 25 Vanadium | 0.01 to 0.50 |

25 with the usual percentages of sulphur and phosphorus. The invention further consists in the alloy steel and articles made therefrom herein-after described and claimed.

30 Our alloy steel is suitable for such articles as valve parts used in high temperatures, oil lines, high temperature steam lines, stay rods in stills and boilers, bolts for high temperature applications and castings and forgings for valve bodies, 35 and other similar articles.

It is recognized that chromium-tungsten-silicon steels have been used as tool steels in the manufacture of such tools as drills, taps, reamers and chisels; but such prior steels have not 40 been satisfactory for use in the articles herein set forth or at high temperatures.

The range of ingredients of our alloy steel is as follows:

|             | Per cent     |
|-------------|--------------|
| 45 Carbon   | 0.20 to 0.60 |
| Manganese   | 0.20 to 1.0  |
| Silicon     | 0.50 to 1.0  |
| Chromium    | 0.75 to 1.50 |
| Tungsten    | 0.75 to 1.50 |
| 50 Vanadium | 0.01 to 0.50 |

A preferred narrower range of ingredients is:

|              | Per cent     |
|--------------|--------------|
| Carbon       | 0.40 to 0.50 |
| 55 Manganese | 0.40 to 0.60 |
| Silicon      | 0.60 to 1.0  |
| Chromium     | 0.75 to 1.25 |
| Tungsten     | 0.75 to 1.0  |

Vanadium in amounts from 0.01 to 0.50% may 60 be used in said steel, the vanadium improving

the properties of the steel at high temperatures. Preferably the tungsten content is substantially smaller in amount than the chromium, sometimes being as little as one-half the chromium content.

5 Tests of numerous specimens of steel within the above range have shown such steels to be resistant to oxidation at high temperatures, to have a high proportional limit value at high temperatures, to have high creep resistance and 10 load carrying ability, to have a high degree of strength, a suitable amount of ductility and good resistance to shock. The steel has an excellent combination of qualities at low or room temperatures, as well as at high temperatures.

### Physical properties at 75° F.

|                 | Tensile strength lbs. per sq. in. | Proportional limit lbs. per sq. in. | Percent elong. 2" | Percent red. area | Bri-nell hardness | Izod impact | 20 |
|-----------------|-----------------------------------|-------------------------------------|-------------------|-------------------|-------------------|-------------|----|
| 130,000-245,000 | 100,000-220,000                   | 6.5-18.0                            | 8.0-54.0          | 270-480           | 20-55             |             |    |

Composition: .39% C, .53% Mn, .68% Si, .84% W, 1.18% Cr

|                 | Tensile strength lbs. per sq. in. | Proportional limit lbs. per sq. in. | Percent elong. 2" | Percent red. area | Bri-nell hardness | Izod impact | 30 |
|-----------------|-----------------------------------|-------------------------------------|-------------------|-------------------|-------------------|-------------|----|
| 140,000-250,000 | 105,000-200,000                   | 6.5-13.0                            | 10.5-40.5         | 270-445           | 9.5-62.5          |             |    |

Composition: .46% C, .47% Mn, .72% Si, .90% W, 1.35% Cr, .30% V

### Physical properties at 1,000° F.

|               | Tensile strength lbs. per sq. in. | Proportional limit lbs. per sq. in. | Percent elong. 2" | Percent red. area | Creep strength 1% per 100,000 hrs. | 40 |
|---------------|-----------------------------------|-------------------------------------|-------------------|-------------------|------------------------------------|----|
| 88,000-95,000 | 24,000-45,000                     | 20-26                               | 78-83             |                   | 7,800                              |    |

Composition: .39% C, .53% Mn, .68% Si, .84% W, 1.18% Cr

|                 | Tensile strength lbs. per sq. in. | Proportional limit lbs. per sq. in. | Percent elong. 2" | Percent red. area | Creep strength 1% per 100,000 hrs. | 45 |
|-----------------|-----------------------------------|-------------------------------------|-------------------|-------------------|------------------------------------|----|
| 114,000-132,000 | 27,000-54,000                     | 17-20                               | 64-71             |                   | 18,000                             |    |

Composition: .46% C, .47% Mn, .72% Si, .90% W, 1.35% Cr, .30% V

55 The qualities and characteristics of our alloy steel as hereinbefore brought out make said steel highly desirable for the uses hereinbefore set forth and in other articles requiring a low priced steel having a good combination of properties at high temperatures and also at low temperatures.

What we claim is:

1. An article, such as a boiler tube or the like, for use at high temperatures the article being

60

formed from a steel alloy characterized by maintained high creep strength under continuous exposure to operating stress at temperatures in excess of 750° F., by substantial resistance to oxidation at operating temperatures, and by containing from more than 0.2 to not more than about 0.6 per cent of carbon, about 0.75 to less than about 1.5 per cent of chromium, about 0.2 to 1.0 per cent of manganese, about 0.5 to 0.9 per cent 5 of silicon, about 0.5 to 1.5 per cent of tungsten, the tungsten content being less than the content of chromium, and the remainder of the steel being substantially iron.

2. An article, such as a boiler tube or the like, 15 for use at high temperatures the article being formed from a steel alloy characterized by maintained high creep strength under continuous exposure to operating stress at temperatures in excess of 750° F., by substantial resistance to oxidation at operating temperatures, and by containing from about 0.4 to 0.5 per cent of carbon, about 0.75 to 1.25 per cent of chromium, about 0.4 to 0.6 per cent of manganese, about 0.6 to 1.0 per cent of silicon, about 0.75 to 1.0 per cent of 20 tungsten, the tungsten content being less than the content of chromium, and the remainder of the steel being substantially iron.

3. An article, such as a boiler tube or the like, 30 for use at high temperatures the article being formed from a steel alloy characterized by maintained high creep strength under continuous exposure to operating stress at temperatures in excess of 750° F., by substantial resistance to oxidation at operating temperatures, and by containing more than 0.2 to not more than about 0.6 per cent of carbon, about 0.75 to less than about 1.5 per cent of chromium, about 0.2 to 1.0 35

per cent of manganese, about 0.5 to 0.9 per cent of silicon, about 0.5 to 1.5 per cent of tungsten, about 0.01 to 0.5 per cent of vanadium, the tungsten content being less than the content of chromium, and the remainder of the steel being substantially iron. 5

4. An article, such as a boiler tube or the like, 10 for use at high temperatures the article being formed from a steel alloy characterized by maintained high creep strength under continuous exposure to operating stress at temperatures in excess of 750° F., by substantial resistance to oxidation at operating temperatures, and by containing from about 0.4 to 0.5 per cent of carbon, about 0.75 to 1.25 per cent of chromium, about 0.4 to 0.6 per cent of manganese, about 0.6 to 1.0 per cent of silicon, about 0.75 to 1.0 per cent of tungsten, about 0.01 to 0.5 per cent of vanadium, the tungsten content being less than the content of chromium, and the remainder of the steel be- 20

5. An article for use at high temperatures the article being formed from a steel alloy characterized by maintained high creep strength under continuous exposure to operating stress at temperatures in excess of 750° F., by substantial resistance to oxidation at operating temperatures, and by containing about 0.46 per cent of carbon, about 1.35 per cent of chromium, about 0.47 per cent of manganese, about 0.72 per cent of silicon, about 0.9 per cent of tungsten, about 0.3 per cent of vanadium, and the remainder of the steel be- 25

ing substantially iron.

WALTER G. HILDORF.

ALBERT E. WHITE.

CLAUDE L. CLARK.

35